

## UNITED STATES PATENT OFFICE.

GEORGE A. RICHTER, OF BERLIN, NEW HAMPSHIRE, ASSIGNOR TO BROWN COMPANY, OF BERLIN, NEW HAMPSHIRE, A CORPORATION OF MAINE.

## WOOD FIBER FOR HIGH-GRADE PAPER AND DERIVATIVE MANUFACTURE.

No Drawing.

Application filed November 7, 1924. Serial No. 748,502.

This invention has for its object to produce a new product, namely a chemical wood pulp, which by reason of its characteristics is capable of uses to which commercial wood pulp 5 is not fitted or adapted.

More particularly the object of the present invention is to produce a pulp consisting of cellulose derived from wood characterized by a high alpha-cellulose content comparable 10 with pulp derived from cotton fibers, by its capacity to be "hydrated" when subjected to the usual beating operation, by a minimum content of impurities, such as lignins, resins and pentosans, by softness of texture and 15 high absorbency. A product having these characteristics may be employed in the manufacture of high grade paper where softness of texture, tearing strength and superior folding or flexing qualities are important, 20 and in the manufacture of cellulose esters or products such as viscose, cellulose nitrate and vulcanized fiber (such for example as produced by the use of zinc chloride).

I shall herein describe a process by which 25 unbleached pulp, such as derived from spruce wood by the cooking thereof in an acid sulphite (either sodium or calcium base) or sodium sulphate-sulphite solution, may be so treated as to produce a maximum yield of the 30 product having the characteristics hereinbefore mentioned, at a relatively low cost, whereby the process may be carried on commercially and continuously; but I do not herein claim such process per se, as it forms 35 the subject-matter of the copending application Serial No. 716,154, filed May 27, 1924.

At the present time it is the commercial practice, in the manufacture of high grade 40 paper having the properties to which I have referred, to employ as the raw material new cotton rags, and, in the manufacture of cellulose products or esters such as viscose, cellulose nitrate, etc., to employ raw cotton or cotton 45 "linters" so-called, and consequently the final product in each case is expensive to produce due to the initial high cost of the raw starting material. The characteristics of cotton, which make its use essential, notwithstanding its relatively high cost, are its purity and fiber length. The cellulosic constituents 50 of any raw fiber are usually divided into three groups,—the alpha, the beta and the gamma

cellulose. The beta and the gamma cellulose represent components which are unstable 55 when exposed to light, moisture, oxygen and alkalies; whereas the alpha cellulose is highly resistant to these agencies. Cotton is characterized by a very high alpha cellulose content, say 94% to 98% of its total weight. A 60 high grade sulphite wood pulp, such as previously produced commercially, has an alpha cellulose content ranging from 83% to 86%, and a correspondingly higher beta and gamma cellulose content than are present in 65 cotton. A pulp produced from cotton fiber is further characterized by a low pentosan content, a very low lignin content, and a low resin and wax content. The pentosan content of a raw or bleached cotton fiber ranges from 70 0.4% to 1%, its lignin content is usually less than 0.3%, and the resinous and waxlike constituents amount to about 0.3%, of the total weight. On the other hand, the pentosan content of high grade sulphite pulp varies from 75 3.5% to 5.5%, the lignin content from 0.5% to 3%, and the resinous content from 0.5% to more than 1%. Furthermore the paper produced from such sulphite pulp is relatively 80 harsh and nonabsorbent, and has what is referred to as a "rattle" when a sheet of the paper is shaken. And, moreover, the paper is much less resistant to tearing action and has a less folding endurance than paper made from cotton fiber. Again, because of its high 85 beta and gamma cellulose content, its high lignin, pentosan and resin content,—the pulp and the paper produced therefrom is less stable when subjected to alkali, moisture, light and oxygen, and the pulp itself is not as suitable as cotton for use in the production of such cellulose esters and products as viscose, cellulose nitrate and the like.

The pulp product, which is the subject of the present invention, has the desirable characteristics of cotton, but it differs from cotton in that it has a shorter fiber and consequently requires less manipulation in its conversion into paper, and has the additional very decided advantage over cotton in that its cost 95 to the consumer is only a fraction of the cost of cotton. It is further distinguishable from cotton when subjected to certain tests which I shall hereinafter describe.

I here present a comparative table of the 105 three materials, namely cotton, commercial

bleached sulphite pulp, and my new product derived from sulphite pulp, to wit:—

|                                                  | Cotton    | Sulphite pulp | New product     |
|--------------------------------------------------|-----------|---------------|-----------------|
| 5                                                |           |               |                 |
| Alpha cellulose, %                               | 94-98     | 83-86         | 93.5-96         |
| Beta cellulose, %                                | 2-3       | 7-9           | 2-4             |
| Gamma cellulose, %                               | 2-3       | 7-8           | 2-2.5           |
| Lignin, %                                        | 0.3-      | 0.5-3.0       | 0.3-            |
| Total cellulose, %                               | 99+       | 97-99         | 99+             |
| Copper number                                    | 0.6-2.0   | 3.5-5.5       | 1.0-2.3         |
| 10 Resins, etc., %                               | 0.3±      | 0.5-1.0       | 0.2-0.4         |
| Pentosans, %                                     | 1.5-1.0   | 3.5-5.5       | 1.0-2.4         |
| Fiber length (av.) **                            | m. m.     | 0.5-8 m. m.   | 1.0-1.5 m. m.   |
| Herzberg fiber stain                             | Wine red. | Blue.         | Reddish purple. |
| 15 Soda solubility, % (3% boiling NaOH solution) | 1-20      | 15-30         | Not over 9.     |

\*\* Note.—The fibers of cotton are very long. These long fibers are not suitable for paper making as such and must be reduced in length. Beaten cotton fiber has approximately the same fiber length as beaten stock made from the new fiber herein described.

20 It should be noted that some of the identifying characteristics assigned to cotton fiber may vary outside the limits set forth. For example a drastic bleaching of a cotton rag stock or raw cotton itself will result in an 25 increased copper number and decreased alpha cellulose. A reasonably severe bleaching, however, would not alter the softness of the paper sheet, nor would it change the stain test appreciably.

30 From the foregoing it will be seen that my new product, having as its starting material sulphite pulp derived from wood chips, has practically all of the desirable characteristics of cotton fiber, so far as the manufacture 35 of paper and cellulose esters or products are concerned, but it is distinguishable therefrom and possesses the advantage of a low cost and a shorter fiber length before beating.

In producing a product having the characteristics herein described, I start with unbleached sulphite pulp such as produced by 40 cooking the chips of spruce in an acid calcium bisulphite or equivalent acid solution (e. g., sodium bisulphite) under conditions of heat and pressure for a sufficient time to produce 45 a pulp which is comparable with high grade unbleached pulp such as manufactured at the present time. The starting material is thus derived from wood, and consists of cellulose 50 which has been freed from the encrusted or cementitious materials and contains specks, knots, resins, lignin, pentosan, and a relatively high proportion of beta and gamma celluloses. This starting material is now treated 55 as follows:—It is preferably first treated as about a 10% stock suspension in a solution containing about 1% to 2% hypochlorite, or about 0.3% to 0.6% chlorine, based on the dry weight of fiber, as described in the here- 60 inbefore identified application for patent. Whether or not the raw or unbleached pulp employed as the starting material should be treated with hypochlorite solution or chlorine water before alkaline digestion depends 65 upon the characteristics of such pulp. The

pretreatment may, for example, be omitted when a well-cooked raw pulp is prepared as the starting material by digesting chipped wood, spruce, for example, in a sodium base acid bisulphite liquor having a combined  $\text{SO}_2$  content of about 1% and a free  $\text{SO}_2$  content of about 5%. But if the usual or commercial unbleached sulphite pulp prepared in calcium bisulphite cooking liquors is employed as the raw material, it should be treated as hereinbefore described, with hypochlorite solution or chlorine water before alkaline digestion, as this makes possible the production of a new product having the desirable characteristics hereinbefore given in the table. As stated in 80 the application hereinbefore referred to, the composition or strength of the hypochlorite solution or chlorine water used in the treatment of the raw pulp before alkaline digestion may be varied, depending upon the particular characteristics of the raw pulp being processed, in order to obtain my new product. As further stated in that application, the first consumption of the oxidizing agent, i. e., the hypochlorite solution or chlorine water, is 90 accompanied by a rise in the proportion of alpha cellulose in the pulp, but a critical point is reached at which further consumption of the oxidizing agent is accompanied by a marked decrease in the proportion of the 95 alpha or resistant cellulose content of the pulp. It has been noted that the copper number decreases with the first consumption of the oxidizing agent up to the critical point, and thereafter rises. Consequently, in carrying on the first step of the process, I employ a relatively small amount of oxidizing agent, based on the amount of pulp, and terminate the operation when or before this critical point is reached, that is, or approximately at 105 the critical point. It is then subjected to the action of dilute alkaline solution at the boiling temperature of the solution for a period of from 3 to 5 hours in an open vessel, sufficient heat being supplied to the vessel to 110 maintain the temperature of the contents at the boiling point of the alkaline solution. This solution is preferably one of caustic soda of approximately 0.5% strength. During this treatment the contents of the vessel are 115 continuously agitated to ensure the permeation of the alkaline solution throughout the mass of pulp. As a result of this treatment, the greater part of the less stable cellulose, i. e. the gamma and beta celluloses, is dissolved 120 in the alkaline solution. The lignin, resin, pentosan content is for the greater part also dissolved in the solution. Preferably, of course, before the unbleached or raw pulp is subjected to this treatment, it is screened 125 for the removal of knots and foreign matter resulting from the digestion.

After the treatment with the alkaline solution, the pulp is washed in any suitable washer for the removal of the alkaline liquor and 130

the substances which have been dissolved therein, and, if desired, treated with antichlor so that the pulp is now neutral.

The pulp is now subjected to the bleaching action of an oxidizing agent such as calcium hypochlorite. This bleaching operation removes from the treated fiber the remaining traces of coloring matter and produces a white fiber. This bleaching action is accomplished without a sacrifice of alpha cellulose content in the finished fibers. Consequently to this end I employ a minimum amount of bleach amounting to from 3% to 5% of bleach powder based on the weight of dry fiber thus treated. Preferably, the bleach liquor contains a certain proportion of free alkali, — say, caustic soda or sodium carbonate, as described in the hereinbefore identified application for patent, as this tends to prevent the formation of oxycelluloses during bleaching, and thus to reduce the copper number of the bleached product. The fiber is again washed to free it of reaction products caused by the bleaching operation, and is recovered by the usual wet machine in sheet form. The pulp thus produced possesses the characteristics which I have hereinbefore described.

I present hereinafter a table showing the papermaking characteristics of certain cellulosic fibers, namely, raw or unbleached sulphite pulp, bleached sulphite pulp, bleached new rag pulp, and my new product:

|                                                                       | Raw sulphite pulp | Bleached sulphite pulp | Bleached new rag pulp | New product |
|-----------------------------------------------------------------------|-------------------|------------------------|-----------------------|-------------|
| Time of beating requisite for normal papermaking                      | 3 hrs.            | 2.5-3 hrs.             | 10-12 hrs.            | 7-8 hrs.    |
| Pop test (Mullen) of resulting paper in points per pound basis weight | 60                | 60                     | 70                    | 60          |
| Tearing resistance per basis weight                                   | 130               | 130                    | 300                   | 230         |
| Folding endurance in double folds per basis weight                    | 1                 | 1                      | 20                    | 7-10        |
| Initial color below                                                   | 93                | 103-104                | 110                   | 104-5       |

From the foregoing comparative table, which sets forth certain physical or papermaking characteristics of my new product, and the comparative table preceding it, which sets forth the chemical composition or characteristics of my new product, it will be seen that my new product has papermaking, as well as chemical, characteristics similar to those of a bleached new rag pulp. My new product is clearly distinguishable from cotton fiber, however, not only by stain test but also microscopically. It is further distinguished from cotton, in that it has a higher pentosan content, this characteristic appar-

ently being desirable when my new product is used as a raw material for papermaking, as pentosans, probably owing to their sticky or adhesive qualities, act as a binder and cement the constituent fibers together when made into paper.

In some instances it may be subjected to what I term a super-bleaching, namely the treatment of the fiber with small quantities of chlorine gas dissolved in water for a final improvement in the color of the fiber. This, however, is not necessary where the pulp is to be employed for the production of cellulose esters or other products, but is sometimes desirable where the pulp is to be used in the manufacture of a very white fine paper.

I do not herein claim the subject matter of patent application Serial No. 716,154, filed May 27, 1924, which is concerned with, and has claims directed to, a method of producing a product such as herein described and claimed.

What I claim is:

1. A new article of manufacture, consisting of cellulose wood pulp of high whiteness having among others the following characteristics, to wit: an alpha cellulose content of 93.5% to 96%, a beta cellulose content of 2% to 4%, a gamma cellulose content of 2% to 3%, a pentosan content not exceeding 2.4%, a copper number of 1.0 to 2.3, producing a reddish-purple color when subjected to Herzberg fiber stain, and of a solubility in 3% boiling NaOH solution of not over 9%.

2. A new article of manufacture consisting of wood fiber of high whiteness, having among others the following characteristics, to wit: an alpha cellulose content not less than 93.5%; a pentosan content not exceeding 2.4%; a copper number not exceeding 2.3, of a solubility in 3% boiling NaOH solution of not over 9%, and producing a reddish purple color when subjected to Herzberg fiber stain.

3. A new article of manufacture consisting of a wood fiber possessing the whiteness of new cotton and having, among others, the following characteristics, to wit: an alpha cellulose content of from 93.5% to 96%, a pentosan content of from 1.0 to 2.4, a copper number of from 1.0 to 2.3 of a solubility in 3% NaOH solution of not over 9%, said wood fiber being characterized by papermaking properties similar to those of a new rag halfstock.

In testimony whereof I have affixed my signature.

GEORGE A. RICHTER.